

Patented July 6, 1926.

## UNITED STATES PATENT OFFICE.

SAMUEL E. SHEPPARD, OF ROCHESTER, NEW YORK, ASSIGNOR TO EASTMAN KODAK COMPANY, OF ROCHESTER, NEW YORK, A CORPORATION OF NEW YORK.

PROCESS OF CHANGING THE LIGHT SENSITIVENESS OF PHOTOGRAPHIC EMULSIONS AND INTERMEDIATE USED THEREIN.

No Drawing.

Application filed December 2, 1925. Serial No. 72,811.

This invention relates to processes for changing the light sensitiveness of photographic emulsions. One object of the invention is to provide a process by means of which photographic emulsions may be improved as regards their light-sensitiveness, without impairing the other properties of the emulsion. Another object of the invention is to provide a process in which a potential sensitizer may be incorporated with the materials of the emulsion, and then the sensitizer liberated at the desired time in the emulsion-making process. Other objects will hereinafter appear.

In my prior application 718,410, filed June 6, 1924, for art of light sensitive photographic materials, I have shown that light sensitizing substances may be prepared by suitably extracting certain organic materials. When these substances are incorporated in photographic emulsions, such as those of the gelatino-silver-halid type, they greatly increase the light-sensitiveness of such emulsions.

I have now found that such sensitizing materials may be prepared in a latent form in which they do not have a sensitizing action, and then can be readily changed from such form so that they do have the sensitizing action. I have further discovered that they stay in their latent form, when incorporated with the materials of the emulsions, and may be converted into the active sensitizing form in such emulsions at the desired time.

In the preferred form of my invention the sensitizing substance is combined with an organic group or radical which maintains it in its latent state until it is released from such group or radical. For instance, a mustard oil sensitizer may be combined in a glucoside, in which form it is latent or inactive, as regards sensitizing action.

While the sensitizing substance may be released from the group or radical by different chemical steps, I prefer to do it, particularly in the case of glucosides, by using a hydrolyzing enzyme. I shall now describe one form of my invention by way of illustration, but it will be understood that the invention is not restricted to the details thus given, except as indicated in the appended claims. Since mustard oils and their gluco-

sides are readily prepared and easily treated, I shall refer to them by way of example.

Sensitizing mustard oils are contained in combined or latent form in vegetable bodies, particularly in the seeds of the plants of the order cruciferæ. They occur usually as glucosides, the monose group or radical with which the oil is combined acting to prevent light-sensitizing action.

While these glucosides can be hydrolyzed in various ways, I have found it particularly convenient to hydrolyze them by means of enzymes. The latter can be used in the emulsion itself, without adversely affecting the latter. Moreover suitable enzymes occur in the same plants as the glucosides only in different cells, and can be obtained in suitable form by simple technique.

I may, for example, crush the seeds of black mustard (*Brassica nigra*) and macerate them in hot alcohol (pure ethyl or denatured) which is raised to a boiling point and held at this point for some time. The residue is then extracted with cold water and evaporated down to a relatively small volume. This watery extract is then made slightly acid by the addition of tartaric acid. The liquid is then still further evaporated and extracted with alcohol. The syrup thus obtained is best diluted and neutralized with potassium carbonate in order to prevent decomposition.

The syrup in this form constitutes a latent sensitizer because it contains the sensitizing substance, namely the allyl mustard oil in combination with the monose radical. If this syrup be added to a photographic emulsion, say for instance a gelatino-silver-halid emulsion of the kind described in my above cited prior application, it produces no sensitizing effect. But at the same time it produces no ill effects on the other properties of the emulsion. It can be thus incorporated at any of the stages in the preparation of the emulsion, even the preliminary ones, say in the gelatine for instance.

Finally the emulsion, containing the latent sensitizer, can be greatly speeded up or sensitized by liberating the combined mustard oil, such as allyl isothiocyanate, which is contained in it. This liberation can be done by melting the emulsion, at a temperature preferably under 50° C., and adding to

it a relatively small amount of gelatine containing the enzyme or ferment. Postponement of the sensitizing operation may even be carried so far as to coat the emulsion on its support while it still contains the latent sensitizer, and then overcoat the emulsion with gelatine containing the enzyme. The latter diffuses into the emulsion and liberates the sensitizer, thereby greatly increasing the 10 light sensitiveness.

The enzyme or ferment may be prepared in any preferred way. I may, for example, macerate white mustard seeds (*Sinapis alba*) and extract them with cold water, the extract being evaporated in a vacuum below 40° C. until a syrup is obtained. It is desirable to keep the temperature below that specified, in order to prevent the destruction of the enzyme by heat. Upon adding alcohol 15 to the syrup the enzyme is precipitated out. This alcoholic precipitate keeps its activity for a considerable time, if it is not exposed to too high a temperature or other protein coagulating agents. It may be incorporated 20 in gelatine, and then the mixture utilized to activate the latent sensitizer in the emulsion, as described hereinabove.

When the latent sensitizer, such as a glucoside of an isothiocyanate, is incorporated 25 in a colloid, such as gelatine, before the colloid is made into an emulsion, the product constitutes a valuable and convenient intermediate in the process of making photographic emulsions, particularly silver-halid ones.

The proportion of latent sensitizer can vary; but in the emulsions and in the intermediates it is used in quantities which will 30 yield the amounts of active sensitizer indicated in my hereinabove cited application.

Having thus described my invention, what I claim as new and desire to secure by Letters Patent is:

1. The process of changing the light-sensitivity of a photographic emulsion which 40 comprises incorporating in said emulsion an organic compound in which a sensitizing substance is combined with a group which renders it latent, and thereafter releasing said substance in active form from said compound.

2. The process of increasing the light-sensitivity of a colloid-silver-salt emulsion

which comprises incorporating in said emulsion a compound in which an isothiocyanate 55 is combined with a group which prevents said isothiocyanate from acting as a sensitizer, and thereafter releasing said isothiocyanate from said group, and thereby restoring its sensitizing power. 60

3. The process of increasing the light-sensitivity of a gelatino-silver-halid emulsion which comprises incorporating with the ingredients of said emulsion a glucoside of a mustard oil, and thereafter freeing said 65 mustard oil by acting on said glucoside with a hydrolyzing enzyme.

4. In the process of preparing a light-sensitive colloid-silver-halid emulsion the step of incorporating in said emulsion an organic latent sensitizer. 70

5. In the process of preparing a colloid-silver-halid emulsion the steps of incorporating with the ingredients of said emulsion a latent sensitizer capable of being activated by an enzyme, and incorporating an enzyme in said emulsion to activate said sensitizer. 75

6. In the process of preparing light-sensitive colloid-silver-halid emulsions the steps 80 of incorporating with the ingredients of said emulsions a latent sensitizer capable of being activated by an enzyme, mixing an enzyme with a colloid, and incorporating said mixture of colloid and enzyme into 85 said emulsion to activate said sensitizer.

7. As an intermediate in the manufacture of colloid-silver-halid emulsions, a colloid having distributed therein particles of silver-halid and a latent organic sensitizer. 90

8. As an intermediate in the manufacture of gelatino-silver-halid emulsions, gelatine having distributed therein minute particles of silver-halid and a sensitizing compound kept in latent form by combination with an 95 organic group.

9. An intermediate in the manufacture of gelatino-silver-halid emulsions comprising gelatine having distributed therein minute particles of silver-halid and a latent sensitizer comprising a compound from which mustard oil can be released by means of an 100 enzyme.

Signed at Rochester, New York, this 25th day of November 1925.

SAMUEL E. SHEPPARD.